

# United States Patent [19]

Sawyer, Jr.

[11] Patent Number: **4,505,716**

[45] Date of Patent: \* Mar. 19, 1985

[54] COMBUSTIBLE COAL/WATER MIXTURE FOR FUELS AND METHODS OF PREPARING SAME

[75] Inventor: **Edgar W. Sawyer, Jr., Hagerstown, Md.**

[73] Assignee: **ITT Corporation, New York, N.Y.**

[\*] Notice: The portion of the term of this patent subsequent to Feb. 21, 2001 has been disclaimed.

[21] Appl. No.: **580,513**

[22] Filed: **Feb. 15, 1984**

[51] Int. Cl.<sup>3</sup> ..... **C10L 1/32**

[52] U.S. Cl. ..... **44/51; 406/197**

[58] Field of Search ..... **44/51; 406/197**

## [56] References Cited

### U.S. PATENT DOCUMENTS

|           |         |             |       |       |
|-----------|---------|-------------|-------|-------|
| 3,628,925 | 12/1971 | Milner      | ..... | 44/51 |
| 3,630,696 | 12/1971 | Milner      | ..... | 44/51 |
| 3,907,134 | 9/1975  | Metzger     | ..... | 44/51 |
| 4,062,694 | 12/1977 | Sawyer, Jr. | ..... | 44/51 |
| 4,104,035 | 8/1978  | Cole et al. | ..... | 44/51 |

|           |         |                  |       |       |
|-----------|---------|------------------|-------|-------|
| 4,147,519 | 4/1979  | Sawyer, Jr.      | ..... | 44/51 |
| 4,162,143 | 7/1979  | Yount            | ..... | 44/51 |
| 4,217,109 | 8/1980  | Siwersson et al. | ..... | 44/51 |
| 4,242,098 | 12/1980 | Braun et al.     | ..... | 44/51 |
| 4,251,230 | 2/1981  | Sawyer, Jr.      | ..... | 44/51 |
| 4,252,540 | 2/1981  | Yamamura et al.  | ..... | 44/51 |
| 4,282,006 | 8/1981  | Funk             | ..... | 44/51 |
| 4,297,107 | 10/1981 | Boehmke          | ..... | 44/51 |
| 4,375,358 | 3/1983  | Swartz et al.    | ..... | 44/51 |
| 4,432,771 | 2/1984  | Sawyer, Jr.      | ..... | 44/51 |

*Primary Examiner*—Y. Harris-Smith

*Attorney, Agent, or Firm*—James B. Raden

## [57] ABSTRACT

Combustible fuel slurry compositions and methods for producing such compositions. The compositions comprise mixtures of particulate coal, water, wetting/dispersing agents for the coal and suspending agents for stabilizing the slurries. The suspending agents include clays such as attapulgite, sepiolite, bentonite and montmorillonite. The wetting/dispersing agents include anionic and non-ionic surface active agents.

39 Claims, No Drawings

**COMBUSTIBLE COAL/WATER MIXTURE FOR FUELS AND METHODS OF PREPARING SAME**

**BACKGROUND OF INVENTION**

This invention relates to a unique fuel and more particularly to a fuel comprising a mixture of finely ground coal, water, a wetting/dispersing agent and a suspending agent.

It has long been known that the present supply of oil is rapidly being depleted. Because of the possible future world shortage of oil and the current price increases in petroleum products, the use of oil as a source of energy has become very expensive, while as indicated above, the supply has an uncertain future. The prior art cognizant of such problems attempted to alleviate the demand for fuel oils by substituting other types of fossil fuels. The abundance of coal and its ready accessibility suggested a direct substitution of coal for oil in many applications. Hence considerable effort has been expended in formulating mixtures of oil and finely ground coal in the ratio of 50 percent oil/50 percent coal to 70 percent oil/30 percent coal.

Examples of typical formulations and techniques are depicted in U.S. Pat. No. 4,147,519 entitled Coal Suspensions in Organic Liquids issued on Apr. 3, 1979 to Edgar W. Sawyer, Jr. the inventor herein and assigned to this assignee.

This Patent describes coal dust powder suspended in fuel oil and stabilized against sedimentation by an additive that makes the mixtures viscous under conditions of low shear while exhibiting low viscosity under high shear conditions to facilitate pumping through long range pipelines by the combination of a suitable surfactant with a gelling grade clay as a suspending agent.

U.S. Pat. No. 4,251,230 entitled Coal Suspensions in Organic Liquids issued on Feb. 17, 1981 to E. W. Sawyer, Jr. describes a suspension of coal dust powder in fuel oil, which suspensions are also stabilized using a gelling grade clay suspending agent.

Other Patents are U.S. Pat. No. 4,062,694 entitled Stable Particulate Suspensions which issued on Dec. 13, 1977 to E. W. Sawyer, Jr. and describes the use of attapulgite clay as a suspending agent for coal dust in flammable liquid hydrocarbons to formulate fuels which facilitate the removal of fly ash from the fuel assembly after burning. As indicated such prior art as well as other Patents, such as U.S. Pat. No. 2,397,859 entitled Liquid Fuel and Method of Producing the Same issued on Apr. 2, 1946 to A. B. Hersberger, et al. attempt to substitute coal for a portion of the oil and provide a composite fuel.

U.S. Pat. No. 4,062,694 also describes coal dust-water slurries that exhibit good rheological characteristics and are useful for transporting and storing coal at a 60% concentration. The slurry is formed using coal, a wetting/dispersing agent for the coal and 1% to 3% gelling grade clay. The 60% coal concentration did not provide sufficient Btu's for the slurry to be considered a satisfactory fuel. The high water content had to be evaporated and that consumed too much of the heat content. The slurry also contributed to another problem, that being ash content. The 1 to 3% clay level contributed significantly to an unacceptable ash level.

Certain of the mixtures depicted in the prior art have been burnt successfully in certain types of furnaces.

The problem with the oil-coal mixtures is that they still contain fuel oil and do so in considerable percentages as between 50 to 70 percent oil.

It is of course understood that the ideal situation is to completely eliminate oil from the composite fuel. Many present installations are designed for powdered coal combustion and have, due to environmental considerations, been retrofitted to burn oil. However, many of the previously retrofitted installations no longer have the auxiliary room and facilities to receive, store and grind coal and therefore changing back to coal or powdered coal combustion is not possible.

It is therefore an object of the present invention to provide a fuel composition which will allow the use of powdered coal as a fuel in the above-mentioned isolated facilities, thus resulting in substantial savings in cost.

Another object is to provide an improved fuel composition employing powdered coal without any fuel oil to provide an efficient stable and economical alternate fuel composition, as well as economical processes for making the composition.

**SUMMARY OF THE INVENTION**

This invention consists of a composition that can be utilized as a fuel which composition comprises a mixture of coal, water, wetting/dispersing agent for the coal and a suspending agent for stabilizing the slurry. Coal is present in the mixture at the 65 to 70 percent level, with the wetting/dispersing agent for the coal employed in minor, functional percentages, the suspending agents employed are natural or synthetic hydrocolloid polymers, gelling type synthetic or natural minerals, or other agents that exhibit gel properties in the water which constitutes the remainder of the composition formula.

**DETAILED DESCRIPTION OF THE INVENTION**

As indicated the invention consists of a composition for a novel fuel comprising a mixture of finely ground coal, water, a wetting/dispersing agent for the coal and a suspending agent for stabilizing the slurry. As will be ascertained the suspending agent may not be required if a suitable wetting/dispersing agent for the coal is used, if the coal is finely ground, and if the slurry will be used in a relatively short period of time after it has been prepared; for example, within twenty-four hours. If a longer storage time is contemplated a suspending agent is necessary.

Coal as anthracite, semi-anthracite, bituminous as well as semi-bituminous and other coal and semi-coal compositions is first crushed and ground by conventional techniques to a fairly fine powder. Examples of successful grinds which can be employed for the coal powder are

1. 95%-100 mesh, 80%-200 mesh, 65%-325 mesh.
2. 90%-100 mesh, 75%-200 mesh, 52%-325 mesh.
3. 100%-325 mesh (44 microns), 55%-26 microns.

The upper limit on the coal particle sizes is dictated by what will burn in the flame (80 mesh). The amount of coal that can be incorporated into coal/water mixture slurries is a function of the particle size distribution, the particle morphology and the dispersing agents employed. Particle size distribution and particle shape can be established during dry processing or by post processing the slurry with various types of conventional wet-grinding equipment to achieve a change in particle size distribution and a rounding off of particle shapes.

It is desirable to incorporate a maximum amount of coal in the slurry while maintaining rheological characteristics that insure good stability and sprayability in the burner nozzle for combustion.

The maximum solids with coal appears to be about 70 to 75 percent and a satisfactory slurry can only be attained with relatively round particles, a high percentage of fine particles and a dispersing/wetting agent. For any medium to long range stability, a gelling agent that imparts gel properties to the continuous water phase is also required. The gelling agent may be omitted if the coal/water mixture is to be combusted soon after preparation and hence will not be stored.

Dispersant/wetting agents effective in this invention are the so-called anionic surface active agents which are 15 low to non-foaming in water, have a structure that consists of an organic moiety that is substantive to (absorbs on) the coal surface in preference to water and a charged hydrophilic portion that is lyophilic to the continuous water phase. These agents are employed at 20 low concentrations and collect on the coal-water interface. They displace air and water, allow the coal agglomerates to be deflocculated with mild stirring and charge up the coal particles to give minimum viscosities.

Other dispersant/wetting agents which also have been found to be effective in this invention are the so-called non-ionic surface active agents which consist of an organic moiety that is substantive to (absorbs on) the coal surface in preference to water and a hydrophilic portion that is lyophilic to the continuous water phase, 30 the hydrophilic portion being a covalent polar functional group which in solution does not ionize. Exemplary of suitable non-ionic surface active agents effective for use as dispersant/wetting agents in the present 35 invention are non-ionic polyether polyols such as ethylene oxide/propylene oxide block copolymers sold under the tradename Pluradyne ES 7478 (BASF Wyandotte Corporation) and other non-ionic polyalkylene oxides condensates such as those sold under the tradename CW-15 (Diamond Shamrock Corporation).

Many types of coal will only make thick pastes when 40 70 percent coal is blended with 30 percent water but when the dispersant/wetting agent is added, they will thin down to very low viscosity fluids when subjected to 45 mild stirring. The dispersant/wetting agent must not interfere with any gellants that are incorporated to improve stability. Anionic surface active agents that function well as dispersant/wetting agents for coal powders are Lomar D and PW (Diamond Shamrock Co.), sodium salts of condensed naphthylene formaldehyde sulfonates, Tamol N and SN (Rohm & Haas Co.), sodium salts of condensed naphthylene formaldehyde sulfonates; Darvan 1 and Darvan 2 (R. T. Vanderbilt Co.), polymerized sodium salts of alkyl naphthalene sulfonic acid and sodium salts of polymerized substituted benzoid alkyl sulfonic acids respectively, and the series of Daxad wetting dispersing agents (W. R. Grace Co.) which are similar in composition to the Lomars & Darvans. Sodium lignosulfonates such as the Rayligs (ITT-Rayonier Co.), the Maracarbs & Marasperses (American Can Co.), Norligs (American Can Co.) and other lignosulfonates can be used.

With regard to usage of non-ionic surface active agents as dispersant/wetting agents herein, it should be noted that addition of such agents tends to result in formation of a foam in the slurry. In order to minimize or eliminate such foam when the non-ionic agents are

utilized, it has been found to be necessary to include a minor, functional amount of a defoaming agent into the slurry during production thereof, preferably in an amount of at least 0.0001% but not in excess of about 5 0.05% based on the weight of the slurry. Exemplary of suitable defoamers which have been found to be effective in this invention are hydrocarbon oil based water dispersible non-ionic surfactants containing hydrophobic colloidal silica such as those sold under the tradename Colloid 642 (Colloid, Inc.) and mixtures of polyglycol fatty esters and polyglycols such as those sold under the tradename Colloid 999 (Colloids, Inc.) Stabilizing agents that maintain the coal powder in suspension in the continuous water phase act through gelling the water phase. The gelled water phase plus the suspended coal should exhibit a gel strength which reversibly breaks under shear so the coal/water mixture (C/WM) can be forced through a burner nozzle to make a burnable spray. Gelling agents that are employed are colloidal grades of Wyoming bentonite, attapulgite, sepiolite, montmorillonites and synthetic smectite clays and gums and other hydrocolloids as carboxyl polymethylene (Carbopol, B. F. Goodrich Co.), carboxymethyl celluloses, alginates, xanthan gums, starches, guar gums, ethoxylated celluloses, and derivatives of these materials.

When clays are employed as suspending agents, they can be predispersed with a chemical dispersant such as TSPP (tetrasodium pyrophosphate) prior to use; for example, with attapulgite clay a predispersion would be:

|             |        |
|-------------|--------|
| Water       | 74.25% |
| TSPP        | 0.75%  |
| Attapulgite | 25.00% |

The resultant predispersion is thin and pourable and can be added to the water of the coal water mixture (C/WM) prior to adding the coal dispersant and coal solids. Montmorillonite can be made up at 30 percent clay solids with 3 percent TSPP, based on the clay weight.

Sepiolite can be made up in a mixture similar to the predispersed attapulgite. Wyoming bentonite is predispersed at the 10 percent clay level with 0.5 percent TSPP. Coal water mixtures containing reflocculated predispersed clays are very stable, have higher gel strengths than those containing gels made from dry clays and are pseudoplastic.

When hydrocolloids are used as stabilizers, their breakdown would be by conventional means as known by those skilled in the art.

In order to gain a still clearer understanding of the 55 composition and the problems attendant with the formulations as well as important data to enable those skilled in the art to provide the composition with a minimum of effort, examples as well as technical considerations will be discussed.

If clays such as attapulgite, sepiolite and Wyoming bentonite are used to stabilize the coal water mixture (C/WM), they can be added to the mix (1) in the final concentration as a dry clay, (2) prehydrated by pregelling in water at a higher concentration and then adding to the slurry at the desired level or (3) predispersed at a high concentration in water using a chemical dispersant and then added to the slurry as a predispersion. If option #3 is used it may be necessary to add a flocculant or

dispersant neutralizer to allow the clay particles to interact and form a stabilizing gel structure.

Typical pregel compositions are:

| Formulations in Parts by Weight |       |       |     |
|---------------------------------|-------|-------|-----|
|                                 | 1     | 2     | 3   |
| Water                           | 85-90 | 85-90 | 90  |
| <u>Clay</u>                     |       |       |     |
| Attapulgite                     | 10-15 | —     | —   |
| Sepiolite                       | —     | 10-15 | —   |
| Wyoming Bentonite               | —     | —     | 10  |
| Total                           | 100   | 100   | 100 |

They are prepared by adding the water to a mixing tank, adding the clay while stirring and continuing agitation until a gel is formed and no clay lumps are present. Pregels are added to a coal/water slurry by addition of the desired aliquot to the water or to the final mix.

Typical predisposition formulations are given below:

| Formulations in Parts by Weight    |        |        |        |
|------------------------------------|--------|--------|--------|
| Water                              | 74.25  | 74.25  | 89.50  |
| Chemical Dispersant<br>(i.e. TSPP) | 0.75   | 0.75   | 0.50   |
| <u>Clay</u>                        |        |        |        |
| Attapulgite                        | 25.00  | —      | —      |
| Sepiolite                          | —      | 25.00  | —      |
| Wyoming bentonite                  | —      | —      | 10.00  |
|                                    | 100.00 | 100.00 | 100.00 |

They are prepared by dissolving the TSPP (Tetrasodium pyrophosphate) in water in a mixing tank, adding the clay while agitating and continuing to agitate until the clay is dispersed. Predispersions of clay can be added at an early or late stage in the C/WM processing but are generally added prior to the coal. Usable chemical dispersants are TSPP, STP (sodium tri-polyphosphate), Calgon, other condensed phosphate dispersants and other polyanionic organic dispersants that function as clay dispersants. Aluminum, magnesium and calcium montmorillonites of the non-swelling varieties (non-gelling grades) can be used as stabilizers in this invention. They can not be added dry or pre-gelled because they develop little viscosity but they will develop gel structures and viscosity if predispersed first and added as a predisposition. A typical predisposition formulation is shown below:

| Parts by Weight |       |
|-----------------|-------|
| Water           | 69.0  |
| TSPP            | 1.0   |
| Ochlocknee Clay | 30.0  |
|                 | 100.0 |

It is prepared as described above and added in the same manner as the other predispersions.

All predispersed clay-stabilized C/WM's should be examined to determine if a dispersant neutralizer is necessary. If a very clean coal is used and the viscosity and gel strength of the final C/WM is low, neutralizers such as hydrated lime, ammonium nitrate, aluminum sulfate, etc., can be added to the final mix to thicken it by floccing the clay component. With dirtier coals there is enough clay present to absorb some of the dispersant;

thus, a gel is produced without the addition of a neutralizer.

Normally the efficiency of clay utilization in suspension stabilization is predispersed pre-gelled dry addition. The same efficiency of usage has been noted in C/WM's.

Examples of the utilization of this invention are shown as follows using a finely ground (80% minus 200 mesh) Kentucky bituminous coal and medium-shear (Sterling Multimixer) processing.

#### EXAMPLE 1—Coal-Water

|       | A    | B    | C    |
|-------|------|------|------|
| Coal  | 70%  | 60%  | 55%  |
| Water | 30%  | 40%  | 45%  |
|       | 100% | 100% | 100% |

1-A This mix was too thick and dilatant.

1-B Thick but pourable. Settled rapidly.

1-C Good consistency but settled out immediately.

#### EXAMPLE 2—Water, Coal, Clay

|             | A    | B      | C    | D      |
|-------------|------|--------|------|--------|
| Water       | 29%  | 29.5%  | 39%  | 44.5%  |
| Attapulgite | 1%   | 0.5%   | 1%   | 0.5%   |
| Coal        | 70%  | 70.0%  | 60%  | 55.0%  |
|             | 100% | 100.0% | 100% | 100.0% |

  

|  | Storage Stability<br>Brookfield Visc. (cP) | Initial, 10/100 RPM | 24 Hrs., 10/100 RPM |                                           |
|--|--------------------------------------------|---------------------|---------------------|-------------------------------------------|
|  |                                            | Too Thick           | Too Thick           | 10,000/<br>8000                           |
|  |                                            | —                   | —                   | 2400/620<br>3000/1250<br>Some<br>settling |

Example 1 formulation results indicate that high coal concentrations (60% to 70%) are thick in consistency and tend to settle. At 55% coal-45% water, they are thinner and settle more rapidly as was the case with 1C.

When attapulgite clay was added, as shown in Example 2, slurries got thicker (2A, 2B and 2C) but the clay stabilized lower concentrations of coal in water in Formulations 2D.

Since 55% coal in water is less desirable than 70% coal in water for combustion purposes, evaluations of coal dispersants/wetting agents were made. Non-ionic dispersant/wetting agents such as ethoxylated castor oil (Surfactol 365), an acetylenic alcohol (Surfynol 104E), an ethoxylated acetylenic alcohol (Surfynol 465) and anionic dispersant/wetting agents such as citric acid were tried and were not effective coal dispersant/wetting agents at higher coal loading levels and, particularly at coal levels in the slurry of greater than 65%. Lignosulfonates and salts of naphthylene formaldehyde sulfonate condensates were good dispersant/wetting agents. They were evaluated with the formulations shown in Example 3 where Raylig 260LR is a 50% sodium lignosulfonate solution, Lomar D is a sodium salt of a condensed naphthylene sulfonate. TSPP is tetrasodium pyrophosphate and Calgon is the sodium salt of a condensed phosphate dispersant.

#### EXAMPLE 3—Water, Coal, Dispersants

|       | A   | B     | C     | D     |
|-------|-----|-------|-------|-------|
| Water | 26% | 29.5% | 29.5% | 29.5% |

-continued

|                              | A             | B             | C         | D         |
|------------------------------|---------------|---------------|-----------|-----------|
| <u>Dispersant</u>            |               |               |           |           |
| Raylig 260LR                 | 4%            | —             | —         | —         |
| Lomar D                      | —             | 0.5%          | —         | —         |
| TSPP                         | —             | —             | 0.5%      | —         |
| Calgon                       | —             | —             | —         | 0.5%      |
| Coal                         | 70%           | 70.0%         | 70.0%     | 70.0%     |
|                              | 100%          | 100.0%        | 100.0%    | 100.0%    |
| <u>Storage Stability</u>     |               |               |           |           |
| <u>Brookfield Visc. (cP)</u> |               |               |           |           |
| Initial                      |               |               |           |           |
| 10/100 RPM                   | 1900/1210     | 3600/1740     | Too thick | Too thick |
| 24 hrs.                      |               |               |           |           |
| 10/100 RPM                   | 1200/750      | 3500/200      | —         | —         |
| 48 hrs.                      | Some settling | Some settling |           |           |

In Example 3, formulations and evaluation results are shown for water-coal-dispersant compositions. Using Raylig 260LR or Lomar D the powdered coal dispersed in water at the 70% level and low viscosities resulted. These two compositions, Formulations 3A and 3B were attractive viscosity-wise but after 24 hours storage showed a slight amount of settling. This resulted from (1) the large coal particles and (2) the fact that no stabilizing gelling agent was present.

Note: TSPP and Calgon did not disperse the coal in water.

Formulations in Example 4 were made to show the effect of dry clay incorporations into Example 3 compositions.

By referring to viscosity results it is noted that attapulgite clay substantially increased the viscosity of the Raylig formulation (4A) but stabilized it against settling. The clay had less of an adverse viscosity effect with the

5 Lomar D formulation, 4E, and it maintained its lower viscosity while remaining stable. Clay in the TSPP- and Calgon-dispersed formulations, 4C and 4D, resulted in compositions that were excessively thick. These formulations were all at the 70% coal level. When the coal 10 concentration was decreased to 65% as in 4B and 4F, much lower viscosities resulted and the formulations were stable.

15 Since normally predispersed attapulgite is more efficient as a suspending agent than dry clay, a 25% predispersion was made up and evaluated in the 70% coal slurry formulations shown in Example 5. Note that the clay is shown as percentage of PD clay and must be divided by four to determine dry clay content.

20 When the formulations and results from Example 5 are considered, it is noted that the amount of predispersed (PD) clay required to stabilize the 70% coal slurries was decreased substantially over that shown in Example 4—the 0.75% PD clay of Formulation 5-A is actually 0.19% dry clay. Raylig 260LR plus PD clay 25 gave formulations that thickened on storage. Lomar D, Lomar PW and Darvan #1, all sodium salts of naphthylene formaldehyde sulfonate condensates, plus PD clay formulations had good viscosities and stabilities.

25 To demonstrate the effects of post processing those slurries, Formula F from Example 5 was made up on a larger scale in a one-gallon Waring Blender. It was then ball milled for 5, 10 and 15 minutes as shown in Example

| Example 4 - Water, Coal, Dispersant, Dry Clay |             |           |                 |           |           |           |
|-----------------------------------------------|-------------|-----------|-----------------|-----------|-----------|-----------|
|                                               | A           | B         | C               | D         | E         | F         |
| Water                                         | 25.5        | 30.5      | 29.0            | 29.0      | 28.9      | 33.9      |
| Dispersant:                                   |             |           |                 |           |           |           |
| Raylig 260LR                                  | 4.0         | 4.0       | —               | —         | —         | —         |
| Lomar D                                       | —           | —         | —               | —         | 0.6       | 0.5       |
| Calgon                                        | —           | —         | 0.5             | —         | —         | —         |
| TSPP                                          | —           | —         | —               | 0.5       | —         | —         |
| Coal                                          | 70.0        | 65.0      | 70.0            | 70.0      | 70.0      | 65.0      |
| Attapulgite                                   | 0.5         | 0.5       | 0.5             | 0.5       | 0.5       | 0.6       |
| Total                                         | 100.0       | 100.0     | 100.0           | 100.0     | 100.0     | 100.0     |
| Storage Stability                             |             |           |                 |           |           |           |
| <u>Brookfield Visc. (cP)</u>                  |             |           |                 |           |           |           |
| Initial                                       | 12,000/4150 | 3000/1300 | 12,000/3600     | Too Thick | 7000/1880 | 4000/1940 |
| 10/100 RPM                                    |             |           |                 |           |           |           |
| 24 hrs                                        | 10,500/4150 | 2300/1510 | 10,000/3750     | —         | 4100/2000 | 4100/1260 |
| 10/100 RPM                                    | No sed.     | No. Sed.  | No sed.         | —         | —         | No sed.   |
| 1 week                                        | —           | —         | Settling & Sed. | —         | —         | 2150,930  |
| 10/100 RPM                                    |             |           |                 |           |           | No sed.   |
| 2 weeks                                       | —           | —         | —               | —         | —         | —         |
| 10/100 RPM                                    |             |           |                 |           |           |           |
| 1 Month                                       | 11,000/4550 | 5000/2040 | —               | —         | —         | —         |
| 10/100 RPM                                    | No sed.     | Sl. sed.  |                 |           |           |           |

| Example 5 - Water, Coal, Dispersant, Predispersant Attapulgite |         |        |         |         |         |         |
|----------------------------------------------------------------|---------|--------|---------|---------|---------|---------|
|                                                                | A       | B      | C       | D       | E       | F       |
| Water                                                          | 25.25%  | 26.4%  | 28.71%  | 28.71%  | 28.65%  | 28.65%  |
| Dispersant:                                                    |         |        |         |         |         |         |
| Raylig 260LR                                                   | 4.0     | 3.0    | —       | —       | —       | —       |
| Lomar D                                                        | —       | —      | 0.54    | —       | —       | 0.6     |
| Lomar PW                                                       | —       | —      | —       | 0.54    | —       | —       |
| Darvan #1                                                      | —       | —      | —       | —       | 0.6     | —       |
| PD Clay (25%)                                                  | 0.75    | 0.6    | 0.75    | 0.75    | 0.75    | 0.75    |
| Coal                                                           | 70.00   | 70.0   | 70.00   | 70.00   | 70.00   | 70.00   |
| Total                                                          | 100.00% | 100.0% | 100.00% | 100.00% | 100.00% | 100.00% |

-continued

## Example 5 - Water, Coal, Dispersant, Predispersant Attapulgite

|                              | A           | B           | C           | D                   | E            | F         |
|------------------------------|-------------|-------------|-------------|---------------------|--------------|-----------|
| <b>Storage Stability</b>     |             |             |             |                     |              |           |
| <u>Brookfield Visc. (cP)</u> |             |             |             |                     |              |           |
| Initial                      | 4800/2220   | 7800/2720   | 4800/2100   | 5200/2220           | 7400/2640    | 5200/2100 |
| 10/100 RPM                   |             |             |             |                     |              |           |
| 24 hrs.                      | 5600/3240   | 6600/2500   | —           | 4400/2180           | 5800/2580    | 4200/2160 |
| 10/100 RPM                   |             |             |             |                     | No sed.      | No sed.   |
| 3 days                       | 12,500/3400 | 7200/3760   | 4600/2020   | 4400/1960           | 7200/2420    | 3900/1800 |
| 10/100 RPM                   | No sed.     | No sed.     | No sed.     | No sed.             | No sed.      | No sed.   |
| 4 days                       | —           | 7200/3560   | —           | —                   | —            | —         |
| 10/100 RPM                   |             | No sed.     |             |                     |              |           |
| 1 week                       | —           | 7600/2940   | 4400/2000   | 3500/1880           | 5200/2280    | 4000/1940 |
| 10/100 RPM                   |             | No sed.     | No sed.     | Very light sediment | Sl. Sed.     |           |
| 1 month                      | —           | 12,000/3900 | 5000/2500   | 4000/1980           | 5200/2600    | —         |
| 10/100 RPM                   |             | No sediment | No sediment | No sediment         | Sl. sediment |           |

## EXAMPLE 6—Effect of Ball Milling to Change Particle Size Distribution and Shape.

20

-continued

| A. Starting formula - Waring Blender processed.       |          |         |                    |
|-------------------------------------------------------|----------|---------|--------------------|
| Water                                                 | 28.65%   |         |                    |
| Lomar D                                               | 0.60     |         |                    |
| PD Clay (25% Clay)                                    | 0.75     |         |                    |
| Coal                                                  | 70.00    |         |                    |
|                                                       | 100.00%  |         |                    |
| <b>Storage Stability</b>                              |          |         |                    |
| Viscosities after Ball Milling (Brookfield Visc., cP) |          |         |                    |
| Ball Milling Time, min.                               | 0        | 5       | 10                 |
| Initial                                               |          |         |                    |
| 10/100 RPM                                            | 1500/580 | 950/925 | 3900/870           |
| 24 hrs.                                               | —        | —       | Paste              |
| 10/100 RPM                                            | —        | —       | 2000/1280          |
| 36 hrs.                                               | —        | —       | —                  |
| 10/100 RPM                                            | —        | —       | 1950/710           |
|                                                       |          |         | No sed.            |
| 1 week                                                | —        | —       | 2000/1640          |
| 10/100 RPM                                            |          |         | No sed., Trace SN* |

SN = supernatant liquor

Ten minute ball milling of formulation 6A resulted in an increase in viscosity over the control but a much smoother looking slurry. Note that the viscosity dropped and became quite stable.

Montmorillonite clay of the non-gelling type can also be used to stabilize C/WM. To demonstrate this a 30% predispersant of montmorillonite clay (PDM) was made up using the formula previously described. The PDM was used in the following 70% coal slurries.

## EXAMPLE 7

|                          | A           | B           |
|--------------------------|-------------|-------------|
| Water                    | 20%         | 13%         |
| Raylig 260LR             | 5           | 7           |
| PDM (30%)                | 5           | 10          |
| Coal                     | 70          | 70          |
|                          | 100%        | 100%        |
| <b>Storage Stability</b> |             |             |
| Brook. Visc. (cP):       |             |             |
| Initial, 10/100 RPM      | 5600/1940   | 9800/2400   |
| 24 hrs., 10/100 RPM      | 6400/2760   | 10,500/3650 |
| 36 hrs., 10/100 RPM      | 6500/2400   | 9500/3100   |
| 1 week, 10/100 RPM       | 6600/3000   | 9600/3500   |
| 1 month, 10/100 RPM      | 13,000/4100 | 14,500/4250 |
|                          | No settling | No settling |

25 The use of 5% of 30% PDM is equivalent in amount of 1.5% dry clay.

It can be concluded from these formulation data and stability results that stable 70% coal-in-water slurries can be made up by employing lignosulfonate dispersants at the 1% to 5% level or sodium salts of naphthalene formaldehyde sulfonate condensate dispersants at the 0.5 to 2.0% level plus attapulgite clay in the dry, pre-gelled or predispersed form as a stabilizer or predispersed non-gelling montmorillonite clay as a stabilizer. If the coal slurry is to be used immediately the clay or other gelling agents will not be necessary to maintain suspension stability.

## EXAMPLE 8

30 A 25% predispersant having the following formulation was prepared utilizing a fine particle size colloidal attapulgite clay:

|             | Percent by Weight |
|-------------|-------------------|
| Water       | 74.25             |
| TSPP        | 0.75              |
| Attapulgite | 25.00             |
|             | 100.00            |

50 Utilizing this predispersant, an 800 g. batch of 70% coal slurry in water was prepared using a high-torque, medium shear laboratory drill press mixer. The coal used was a 200 mesh, 13,905 Btu/lb. Consol Coal Company boiler coal with an ash of 7.2% and ASTM ash fusion temperatures of 2320°-2580° F. The coal dispersant used was a flaked nonionic ethylene oxide/propylene oxide block copolymer sold by BASF Wyandotte Corporation under trade name "Pluradyne ES 7478" and was introduced into the slurry as a 10% aqueous solution. The formulation of the slurry was as follows:

|                         | Percent by Weight |
|-------------------------|-------------------|
| Water                   | 23                |
| 25% Predispersant       | 2                 |
| 10% Dispersant Solution | 5                 |
| Coal                    | 70                |

-continued

|  | Percent by Weight |
|--|-------------------|
|  | 100               |

It should be noted in the above formulation that the amount of clay present in the slurry (on a dry weight basis) was 0.5% and the amount of dispersant (on a dry weight basis) was 0.5%. It should be further noted that during preparation of the slurry, a defoamer was added to minimize the foam generated by the nonionic dispersant utilized therein. The amount of defoamer introduced was 0.004% by weight of the slurry and the defoamer employed was a colloidal silica type defoamer sold by Colloids, Inc. under the trade name Colloid 642.

Initial Brookfield viscosities of the resulting slurry were 2700 cP at 10 RPM and 1260 cP at 100 RPM. Stability tests were conducted over a one month period and it was determined that the slurry exhibited good viscosity stability with the appearance of a slight supernatant liquid and no settling of cake on the bottom of the storage container.

#### EXAMPLE 9

Slurries were formulated in accordance with the procedures of Example 8 except that the formulation was scaled-up in pilot plant preparations using a Cowles dissolver mixer (Model W-24, 10 H.P., 9.5 inch mixing blade) at 1000 RPM and a 55 gallon drum as a mix tank. Each slurry batch resulted in 286 lbs. of coal/water suspension and a total of 1716 lbs. were prepared. Evaluation of the large mixes were similar to those achieved with the small batches of Example 8, again demonstrating the good stability characteristics of the slurries over an extended time period.

#### EXAMPLE 10

Utilizing the procedures of Example 6, a coal/water slurry was prepared having the following formulation:

|                   | Percent by Weight |
|-------------------|-------------------|
| Water             | 25.8              |
| 25% Predispersion | 1.0               |
| Dispersant (A-23) | 2.0               |
| Coal              | 71.2              |
|                   | 100.0             |

It should be noted in the above formulation that the amount of clay present in the slurry (on a dry weight basis) was 0.25% and the amount of dispersant (on a dry weight basis) was 1.0% since the dispersant utilized (i.e., A-23) was a 50% solution of ammonium salts of condensed naphthylene formaldehyde sulfonates (Diamond Shamrock).

The storage stability of this formulation was then tested with the following results indicating the effectiveness thereof:

| Storage Stability          |
|----------------------------|
| Brookfield Visc. (cP)      |
| Initial, 10/100 RPM        |
| 24 Hrs., 10/100 RPM        |
| 1 week, 10/100 RPM         |
| no settling<br>no sediment |

#### EXAMPLE 11

Utilizing the procedures of Examples 6, a stable and effective coal/water slurry may be prepared including 5 72% coal (by weight of the slurry) wherein the formulation is as follows:

|                          | Percent by Weight |
|--------------------------|-------------------|
| 10 Water                 | 26.65             |
| 25% Predispersion        | 0.75              |
| 10% Dispersant (Lomar D) | 0.60              |
| Coal                     | 72.00             |
|                          | 100.00            |

15

#### EXAMPLE 12

Utilizing the procedures of Example 8, a stable and effective coal/water slurry may be prepared including 20 72% coal (by weight of the slurry) wherein the formulation is as follows:

|                                    | Percent by Weight |
|------------------------------------|-------------------|
| 25 Water                           | 21.00             |
| 25% Predispersion                  | 2.00              |
| 10% Dispersant (Pluradyne ES 7478) | 5.00              |
| Coal                               | 72.00             |
|                                    | 100.00            |

30

What is claimed is:

1. A combustible fuel slurry comprising: greater than about 70% to about 75% by weight coal powder in particulate form and having a rounded particle shape; from 0.5-5% by weight of a wetting/dispersing agent selected to be low to non-foaming in water and having a structure that consists of an organic portion that absorbs on the surface of said coal particles with said agent having a charged hydrophilic portion that is lyophilic to the continuous water phase; a clay stabilizing composition in the form of a predis-persion comprising a clay stabilizer, a clay dispersant and water wherein the amount of clay stabilizer in the fuel slurry is from 0.15 to 0.8% by weight; and the remainder of said fuel being water, whereby the clay stabilizer, when added to the fuel slurry, provides a stabilizing gel structure for the slurry.
2. The fuel slurry according to claim 1 wherein said particle size is about 80 mesh.
3. The fuel slurry according to claim 1 wherein said wetting/dispersing agent is selected from the group consisting of sodium salts of condensed naphthylene formaldehyde sulfonates, polymerized sodium salts of alkyl naphthylene sulfonic acid, sodium salts of polymerized substituted benzoid alkyl sulfonic acids and sodium lignosulfonates.
4. A combustible fuel slurry as described in claim 1 wherein the clay dispersant is selected from the group consisting essentially of tetrasodium pyrophosphate, sodium tripolyphosphate, condensed phosphate dispersants and sodium salts thereof, and polyanionic organic dispersants that function as clay dispersants.
5. A combustible fuel slurry as described in claim 1 wherein said clay stabilizer is selected from the group

50

55

60

65

consisting essentially of bentonite, attapulgite, sepiolite and montmorillonite.

6. A combustible fuel slurry as described in claim 1 wherein the predispersing comprises from 10-30% by weight clay stabilizer, 0.5-1.0% by weight clay dispersant and the remainder being water. 5

7. A combustible fuel slurry as described in claim 1 additionally including a neutralizer for floccing the dispersed clay component.

8. A method of making a combustible coal/water fuel slurry, comprising the steps of:

preparing a stabilizing composition by adding from 10-15% by weight of a clay selected from the group consisting essentially of attapulgite, sepiolite and Wyoming bentonite to water while both stirring and agitating to form a pregel; 15

adding from 0.5-5% by weight of a wetting/dispersing agent for coal to the water of the fuel slurry; adding said stabilizing composition to said slurry water; and 20

adding greater than about 70% to about 75% by weight coal while stirring to provide a gelled fuel.

9. The method according to claim 8 wherein said coal powder is bituminous coal powder of 200 mesh diameter particles.

10. A method of making a combustible coal/water fuel slurry, comprising the steps of:

preparing a stabilizing composition by adding a clay dispersant and a clay stabilizing agent to water while agitating and continuing to agitate until the 30 clay stabilizing agent is dispersed to form a predispersing;

adding from 0.5 to 5.0% by weight of a wetting/dispersing agent for coal to the water of the fuel slurry;

adding said stabilizing composition to said slurry water; and 35

adding greater than about 70% to about 75% by weight coal while stirring to provide a gelled fuel.

11. The method according to claim 10 including the 40 further step of adding a neutralizer after stirring to thicken the final mix.

12. The method according to claim 11 wherein said neutralizer is selected from hydrated lime, ammonium nitrate, aluminum sulfate. 45

13. A method of making a combustible coal/water fuel slurry as described in claim 10, wherein the wetting/dispersing agent is selected from the group consisting essentially of salts of condensed naphthylene formaldehyde sulfonates, polymerized salts of alkyl naphthylene sulfonic acid, salts of polymerized substituted benzoid alkyl sulfonic acids, salts of lignosulfonates. 50

14. A method of making a combustible coal/water fuel slurry as described in claim 10, wherein the clay dispersant is selected from the group consisting essentially of tetrasodium pyrophosphate, sodium tripolyphosphate, condensed phosphate dispersants and sodium salts thereof, and polyanionic organic dispersants that function as clay dispersants. 55

15. A method of making a combustible coal/water fuel slurry as described in claim 10 wherein the clay stabilizing agent is selected from the group consisting essentially of bentonite, attapulgite, sepiolite and montmorillonite.

16. A method of making a combustible coal/water fuel slurry as described in claim 10 wherein the stabilizing composition is prepared by adding 10 to 30% by weight clay dispersant so that the total clay stabilizing 65

agent in the fuel slurry is from 0.2 to 0.8% by slurry weight.

17. A combustible fuel slurry comprising: from about 65% to about 75% by weight coal powder in particulate form and having a rounded particle shape;

from 0.5-5% by weight of a wetting/dispersing agent selected to be low to non-foaming in water and having a structure that consists of an organic portion that absorbs on the surface of said coal particles with said agent having a charged hydrophilic portion that is lyophilic to the continuous water phase;

a clay stabilizing composition in the form of a pregel comprising a clay stabilizer and water wherein the amount of clay stabilizer in the fuel slurry is from 0.15 to 0.8% by weight; and

the remainder of said fuel being water, whereby the clay stabilizer, when added to the fuel slurry, provides a stabilizing gel structure for the slurry.

18. The fuel slurry according to claim 17 wherein said particle size is about 200 mesh.

19. The fuel slurry according to claim 17 wherein said wetting/dispersing agent is selected from the group consisting of sodium salts of condensed naphthylene formaldehyde sulfonates, polymerized sodium salts of alkyl naphthylene sulfonic acid, sodium salts of polymerized substituted benzoid alkyl sulfonic acids and sodium lignosulfonates. 25

20. A combustible fuel slurry as described in claim 17 wherein said clay stabilizer is selected from the group consisting essentially of bentonite, attapulgite and sepiolite clays.

21. A combustible fuel slurry as described in claim 17 wherein the pregel includes from 10-15% by weight clay stabilizer.

22. A combustible fuel slurry as described in claim 17 wherein said coal powder is bituminous coal powder.

23. A combustible fuel slurry comprising: from about 65% to about 75% by weight coal powder in particulate form and having a rounded particle shape;

from 0.5-5% by weight of a non-ionic surface active wetting/dispersing agent effective for dispersing said percentage of said coal in said slurry, said wetting/dispersing agent having a structure that includes an organic portion that absorbs on the surface of said coal particles with said agent having a hydrophilic portion that is lyophilic to the continuous water phase, said hydrophilic portion being a covalent polar functional group which in solution does not ionize;

a defoaming agent in an amount sufficient to minimize foam formed during production of said slurry; a clay stabilizing composition in the form of a predispersing comprising a clay stabilizer, a clay dispersant and water wherein the amount of clay stabilizer in the fuel slurry is from 0.15 to 0.8% by weight; and

the remainder of said fuel being water, whereby the clay stabilizer, when added to the fuel slurry, provides a stabilizing gel structure for the slurry.

24. The fuel slurry according to claim 23 wherein said particle size is about 80 mesh.

25. The fuel slurry according to claim 23 wherein said wetting/dispersing agent is a non-ionic polyalkylene oxide condensate.

26. The fuel slurry according to claim 25 wherein said wetting/dispersing agent is a non-ionic ethylene oxide/-propylene oxide block copolymer.

27. The fuel slurry according to claim 23 wherein said defoaming agent is incorporated into the slurry in an amount of up to about 0.05% based on the weight of the slurry. 5

28. A combustible fuel slurry as described in claim 23 wherein the clay dispersant is selected from the group consisting essentially of tetrasodium pyrophosphate, sodium tripolyphosphate, condensed phosphate dispersants and sodium salts thereof, and polyanionic organic dispersants that function as clay dispersants. 10

29. A combustible fuel slurry as described in claim 23 wherein said clay stabilizer is selected from the group consisting essentially of bentonite, attapulgite, sepiolite and montmorillonite clays. 15

30. A combustible fuel slurry as described in claim 23 wherein the predispersion comprises from 10-30% by weight clay stabilizer, 0.5-1.0% by weight clay dispersant and the remainder being water. 20

31. A combustible fuel slurry as described in claim 23 additionally including a neutralizer for floccing the dispersed clay component.

32. A combustible fuel slurry comprising:  
from about 65% to about 75% by weight coal powder in particulate form and having a rounded particle shape; P1 from 0.5-5% by weight of a non-ionic surface active wetting/dispersing agent effective for dispersing said percentage of said coal in said slurry, said wetting/dispersing agent having a structure that includes an organic portion that absorbs on the surface of said coal particles with said agent having a hydrophilic portion that is lyophilic 30

25

to the continuous water phase, said hydrophilic portion being a covalent polar functional group which in solution does not ionize;

a defoaming agent in an amount sufficient to minimize foam formed during production of said slurry; a clay stabilizing composition in the form of a pregel comprising a clay stabilizer and water wherein the amount of clay stabilizer in the fuel slurry is from 0.15 to 0.8% by weight; and the remainder of said fuel being water, whereby the clay stabilizer, when added to the fuel slurry, provides a stabilizing gel structure for the slurry. 10

33. The fuel slurry according to claim 32 wherein said particle size is about 200 mesh.

34. The fuel slurry according to claim 32 wherein said wetting/dispersing agent is a non-ionic polyalkylene oxide condensate.

35. The fuel slurry according to claim 34 wherein said wetting/dispersing agent is a non-ionic ethylene oxide/-propylene oxide block copolymer.

36. A combustible fuel slurry as described in claim 32 wherein said clay stabilizer is selected from the group consisting essentially of bentonite, attapulgite and sepiolite clays.

37. A combustible fuel slurry as described in claim 32 wherein the pregel includes from 10-15% by weight clay stabilizer.

38. A combustible fuel slurry as described in claim 32 wherein said coal powder is bituminous coal powder.

39. The fuel slurry according to claim 32 wherein said defoaming agent is incorporated into the slurry in an amount up to about 0.05% based on the weight of the slurry.

\* \* \* \* \*

35

40

45

50

55

60

65